

# United States Patent [19]

Basche et al.

[11] 3,850,689

[45] Nov. 26, 1974

[54] PROCEDURES FOR COATING  
SUBSTRATES WITH SILICON CARBIDE

[75] Inventors: **Malcolm Basche**, West Hartford, Conn.; **Roy Fanti**, Springfield, Mass.

[73] Assignee: **United Aircraft Corporation**, East Hartford, Conn.

[22] Filed: **Apr. 8, 1970**

[21] Appl. No.: **26,556**

**Related U.S. Application Data**

[63] Continuation of Ser. No. 566,098, July 18, 1966, abandoned.

[52] **U.S. Cl.** 117/229, 65/3, 117/93, 117/106 C, 117/115, 117/121, 117/126 AF, 117/126 GF, 117/128, 117/135.1, 117/169 R, 117/231

[51] **Int. Cl.** B32b 15/02, B44d 1/42, C03c 25/02

[58] **Field of Search** 117/93.1, 229, 107.2, 106 C, 117/126 AF, 126 GF, 169 R, 135.1, 128, 121, 93, 115, 231; 65/3

[56] **References Cited**

UNITED STATES PATENTS

|           |         |                |            |
|-----------|---------|----------------|------------|
| 1,987,576 | 1/1935  | Moers          | 117/106 C  |
| 3,083,550 | 4/1963  | Averbach       | 117/107.2  |
| 3,136,799 | 6/1964  | Maginn         | 117/107.2  |
| 3,157,541 | 11/1964 | Heywang et al. | 117/106 C  |
| 3,178,308 | 4/1965  | Oxley et al.   | 117/106 C  |
| 3,212,926 | 10/1965 | Morelock       | 117/126 GF |

3,455,723 7/1969 Kern ..... 117/135.1  
3,554,782 1/1971 Nieberlein ..... 117/135.1

FOREIGN PATENTS OR APPLICATIONS

145,106 4/1962 U.S.S.R. ..... 117/106 C

*Primary Examiner*—William D. Martin

*Assistant Examiner*—William H. Schmidt

*Attorney, Agent, or Firm*—John D. Del Ponti

[57] **ABSTRACT**

Thin, adherent oxidation and corrosion resistant silicon carbide coatings are provided on filamentary base materials by continuously passing a hot surface of the filamentary material through a liquid organo silicon halide, wherein the temperature of the hot surface is high enough to cause the organo silicon halide immediately surrounding the hot surface to film boil, decompose, and deposit the silicon carbide coating. The filamentary base material has a melting point which exceeds the formation temperature of silicon carbide. The base material may be tungsten, tantalum, columbium, or alloys thereof. The base material may also be glass or alumina. When the base material is glass, the glass filaments may be coated directly after forming. All of the substrates may be preheated to the required temperature and the substrates which are electrically conductive may be heated by electrical resistance heating.

15 Claims, 4 Drawing Figures



PATENTED NOV 26 1974

3,850,689

SHEET 1 OF 4

FIG-1



INVENTORS  
MALCOLM BASCHE  
ROY FONTI  
BY  
MORGAN, FINNEGAN, DURHAM & PINE  
ATTORNEYS

PATENTED NOV 26 1974

3,850,689

SHEET 2 OF 4



FIG-2

INVENTORS  
MALCOLM BASCHE  
ROY FONTI  
BY  
MORGAN, FINNEGAN, DURHAM & PINE

ATTORNEYS

PATENTED NOV 26 1974

3,850,689

SHEET 3 OF 4



FIG-3

INVENTORS  
MALCOLM BASCHE  
ROY FONTI

BY  
MORGAN, FINNEGAN, DURHAM & PINE

ATTORNEYS

PATENTED NOV 26 1974

3,850,689

SHEET 4 OF 4



FIG-4

INVENTORS  
MALCOLM BASCHE  
ROY FONTI  
BY  
MORGAN, FINNEGAN, DURHAM & PINE

ATTORNEYS

## PROCEDURES FOR COATING SUBSTRATES WITH SILICON CARBIDE

The present application is a continuation of U.S. application Ser. No. 566,098, filed July 18, 1966, now abandoned, and relates to methods for plating or coating insulating as well as electrically conducting substrata with silicon carbide and also to the plating or coating of filamentary forms of such substrata with silicon carbide.

One object of the present invention is to provide improved procedures for imposing a controlled coating of silicon carbide on both insulating and conducting substrata.

Another object of this invention is to continuously coat substrata of the type described with silicon carbide at high rates, so as to render such substrata resistant to oxidation, contamination and wear.

Another object of this invention is to coat continuous filaments of conducting as well as non-conducting material with silicon carbide.

A further object of the present invention is to produce composite silicon carbide coated filaments having high strength and modulus to weight ratios for use in the fabrication of structural members, including filament wound structures and fibre reinforced structures.

Additional objects and advantages of the invention will be set forth in part as part of the description and drawings which follow and in part will be obvious from the description, or may be learned by practice of the invention, the objects and advantages being realized and attained by means of the compositions, methods and apparatus particularly pointed out in the appended claims.

According to the present invention, a new and improved method has been developed to achieve dense, uniform, adherent, non-porous coatings of silicon carbide under controlled conditions at extremely high rates on a wide variety of insulating and conducting substrata.

According to one embodiment, a suitable substratum is contacted with an organosilicon halide, the temperature of the substratum being sufficiently high to cause decomposition of the organosilicon halide, to thereby deposit silicon carbide on the surface thereof. Thus, according to a preferred embodiment of the invention, a suitable substratum in contact with or prior to contact with an organosilicon halide, is heated to a temperature above the decomposition temperature of the organosilicon halide, i.e., above about 500°C. and preferably above about 800°C., but below the melting point of the substratum, to thereby cause on contact decomposition of the organosilicon halide and simultaneous deposition of silicon carbide on the substratum.

FIG. 1 is a schematic illustration of a suitable bath reactor for carrying out one embodiment of the invention;

FIG. 2 is a schematic illustration of a suitable inclined reactor for carrying out a continuous coating procedure in accordance with another embodiment of the invention;

FIG. 3 shows a schematic illustration of a vertical embodiment of an apparatus which may be used to alleviate the hot spot problem of the FIG. 2 apparatus; and

FIG. 4 shows a schematic illustration of an apparatus suitable for coating glass fibers directly after their formation.

FIG. 1 is a schematic illustration of a suitable bath reactor for carrying out such an embodiment of the invention. A suitable reaction vessel 2, which may for example be made of glass, is suitably sealed with head plate 4 by means of gasket 6. The reaction vessel is filled with a liquid organosilicon halide 8 to the desired level. The head 4 is provided with an exhaust 10 for venting gases released by the decomposition of the organosilicon halide. The reaction vessel 2 is also provided with insulated electrodes 12 and 16 and is submerged in the liquid reactant material 8. The hinged lower grip 20 provides tension to keep the wire 18 straight. The exhaust opening 10 prevents pressure build-up in the reaction vessel and is vented to atmosphere. When the substrata is conducting, voltage, either A-C or D-C, is applied to the electrodes 12 and 16 to heat the substrate above the decomposition temperature of the organosilicon halide. Alternatively, when the substrata is nonconducting, a suitable auxiliary pre-heating device, such as an inductance coil, may be used to heat the substratum to the required temperature. In operation with a conducting substratum, the apparatus of FIG. 1 is filled with a liquid organosilicon compound, for example, methylene dichloride silane ( $\text{CH}_2\text{SiHCl}_2$ ). As sufficient voltage is applied to the wire to heat it to a temperature high enough to cause the liquid reactant to decompose, silicon carbide will deposit as a solid on the hot substrate while gaseous hydrogen chloride will bubble off through port 10. At the end of the run, argon or another inert gas may be bubbled through the hollow electrode 16 to purge the gaseous reaction products from the liquid reactant.

The process is adaptable for coating a wide variety of substrate material, as will be clear from the following examples,

### EXAMPLE 1

Using the apparatus of FIG. 1, a  $\frac{1}{2}$  mil tungsten substrate was coated with silicon carbide. The tungsten filament was attached to electrodes 12 and 16 as shown in FIG. 1 and heated by resistance heater to a temperature of between 900° and 1,500°C. The liquid reactant material was methylene dichloride silane. The plating times and resulting thickness of the deposit were as follows:

| Coating Time | ½ Mil Tungsten Substrate |           | Final Diameter of Wire in Inches |
|--------------|--------------------------|-----------|----------------------------------|
|              | 5<br>Seconds             | 16<br>do. |                                  |
| 16           | do.                      |           | .005                             |
| 20           | do.                      |           | .018                             |
| 22           | do.                      |           | .022                             |
|              |                          |           | .025                             |

X-ray analysis of the silicon carbide coated tungsten wire of Example 1 showed the deposit to be beta silicon carbide, with undetectable amounts of anything else present.

### EXAMPLE 2

Example 1 was repeated except that a 1.8 mil tantalum wire was used as the substratum. Plating time and resulting thicknesses of deposit were as follows:

| 1.8 Mil Tantalum Substrate |  | Final Diameter of Wire in Inches |
|----------------------------|--|----------------------------------|
| Coating Time               |  |                                  |
| 20 Seconds                 |  | .026                             |
| 40 do.                     |  | .041                             |

## EXAMPLE 3

Example 1 was repeated except that an 18 mil stainless steel wire was used as a substratum. Plating times and resulting thicknesses of deposit were as follows:

| 18 Mil Stainless Substrate |  | Final Diameter of Wire in Inches |
|----------------------------|--|----------------------------------|
| Coating Time               |  |                                  |
| 3 Seconds                  |  | .020                             |
| 5 do.                      |  | .024                             |

## EXAMPLE 4

A 2 mm glass rod was heated to a dull red temperature and plunged into liquid methyl dichlorosilane. A 1 mil thick coating of silicon carbide was formed on the glass rod.

Although the procedure using the apparatus of FIG. 1 has been described with reference to the coating of substratum in filament form, it should be understood that using the apparatus described, a silicon carbide coating may be imposed on a suitable substratum of any desired shape to provide protection against wear, oxidation or erosion.

Heating of the object to be coated may be accomplished by self-resistance heating of a substratum in contact with the liquid reactant, or by induction or other suitable pre-heat means, followed by exposure to the liquid reactant. Self-resistance heating is most suitable for wires or ribbons. Large objects could be heated for example by induction coils placed outside the reactor. When large pieces or smaller objects, e.g., wire, are to be coated continuously, it is desirable to circulate the reactant liquid to a cooling chamber, in order to avoid over heating of the reactant liquid.

In any event, when the reactant is liquid, care should be used to maintain the bulk of the liquid below its boiling point to avoid excessive bubbling. It is recognized, however, that at the preferred temperatures, the liquid immediately surrounding the immersed object will boil vigorously and film boiling will be established.

The procedure of the embodiment described has many advantages over conventional pyrolytic processes. Thus, as compared with such conventional techniques, the present procedure requires no metering of any kind of gas and is therefore susceptible of good control. Since extremely high concentrations of reactant material are possible, i.e., a pure or substantially pure organosilicon halide may be used as the reactant fluid, a rapid rate of deposition is assured. Reaction by-products are removed immediately as they form and therefore do not have an opportunity to foul up the system. A further advantage is the fact that stoichiometry is achieved without any metering or control being necessary, and a uniform distribution of reactant material is therefore quite easy to obtain. Thus, parts of any shape can be coated uniformly.

The invention may be used to coat a wide variety of objects, including engine components having improved high temperature capability, e.g., improved oxidation and erosion resistance. Parts subject to severe wear 5 may also be coated in accordance with the present invention to provide high hardness even at elevated temperatures.

The invention is particularly suitable for protecting tungsten, columbium, and tantalum components from 10 decomposition due to oxidizing atmospheres. When applied to the coating of glass, the mechanical properties of the glass are greatly improved.

FIG. 2 is a schematic illustration of a suitable inclined reactor for carrying out a continuous coating procedure in accordance with a further embodiment of the invention. A suitable reaction vessel 50, which may, for example, be made of glass, is suitably sealed with head plates 54 and 56, by means of gaskets 55. The reactor is filled with a liquid organosilicon halide 70. The head 15 55 is provided with an exhaust 66 for venting reaction gases. The head plates 54 and 56 are also provided with insulated electrodes 60 and 64. Electrodes 60 and 64 are preferably hollow and may be filled with a liquid, e.g., mercury, for sealing and/or electrical contact purposes. The substrate to be coated is a continuous wire 20 62 which passes through electrode 60, the liquid reactant 70 and electrode 64 from which it emerges as a silicon carbide coated wire 65. The apparatus of FIG. 2 is especially suitable for coating substrates in the form of 25 wires which are electrically conducting, since such wires can readily be heated by self-resistance. Appropriate feed and take-up reels or other devices may be used to feed and take-up the filament substrate 62 and the coated wire 65, respectively. When the substrate is 30 35 40 45 50 55 60 65 70 75 80 85 90 95 100 the coated wire 65, respectively. When the substrate is 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9

and the current was therefore limited to prevent burn-out in this section. The silicon carbide coated tungsten wire product tested 180,000 psi tensile.

In FIG. 3 is shown a vertical embodiment of an apparatus which may be used to alleviate the hot spot problem encountered with the FIG. 2 apparatus as explained in Example 5.

As shown in FIG. 3, 10 is a cylindrical reactor which may be provided with a suitable cooling jacket 8 having suitable coolant inlet and outlet ports 17 and 18, respectively. Reactor 10 is sealed by upper header assembly 19 and lower heating assembly 20, respectively. The header assemblies are sealed to reactor tube 10 by means of gaskets 15.

Upper header assembly 19 includes an upper mercury inlet tube 1 and an upper electrode and seal jewel assembly 2. Upper liquid or gas port 3 and upper gas exhaust port 5 extend horizontally into upper electrode and seal liquid and gas port assembly 4. Tube 6 is a continuation of upper mercury inlet tube 1 and extends into the chamber within reactor 10. Tube 6 is fitted at its lower end with a removable jewel holding cap 7 which serves to guide the wire 21 being coated. Lower header 20 is provided with a lower mercury electrode 11, and a lower mercury fill tube 12. Also provided is a gas or liquid inlet tube 13 and a removable lower jewel holder 14. The reactor 10 is filled to a suitable level with liquid reactant material 22.

The operation of the FIG. 3 apparatus will be clear from the following examples:

#### EXAMPLE 6

The trouble with the hot spot which developed in the vertical apparatus of FIG. 2 as described in Example 5 was eliminated by using the vertical apparatus of FIG. 3, in which the wire feed-in was at the bottom, thus keeping the hot spot under the liquid at all times. In FIG. 3, the gas port 5 was used to exhaust the produced gas, both HCl, H<sub>2</sub>, etc., as well as vaporized silane. When the water jacket 8 was used (0°C. water circulated in the jacket), the decrease in liquid level was very slow. Additional silane was added through inlet tube 13 from a reservoir and valve system. The methyl dichlorosilane was also directly cooled by circulating it by means of ports 3 and 13 through a copper coil immersed in an ice bath. A small circulatory pump was used for this purpose.

In a 6-inch long reactor tube 10 at 1,125 feet per hour, 1.4 mil silicon carbide filament was produced on a 0.5 mil tungsten substrate with a current of 280 milliamps. The coated material had a tensile strength of 331,000 psi.

#### EXAMPLE 7

In another modification of processing procedure, the vertical reactor of FIG. 3 was run in a combined liquid-gas phase operation. That is to say the liquid methyl dichlorosilane level was kept somewhere below the top jewel 7. This procedure essentially produced a two-stage reactor with a coating being put on in the liquid and another put on in the fully saturated gas above the liquid. The temperature was controlled by adjusting the liquid level and gas input to the top section. At half liquid, half gas, the wire was hotter in the gas section but due to the small amount of SiC deposited from the liquid section, the hot spot problem was eliminated and a very uniform elevated temperature of about 1,500°C.

was maintained in the upper section. In such a combined reactor the exhaust was through port 5 and a stream of H<sub>2</sub> was added at port 3 to keep the jewel 7 clean and cool. Starting with one-half mil tungsten wire, a SiC coated filament 4.2 mils in diameter was produced in a 10 inch long reactor filled with about 4 inches of liquid methyl dichlorosilane at a rate of 103 feet per hour. This filament had a tensile strength of 250,000 to 350,000 psi. At 206 feet per hour a 3.35—3.40 mil SiC coated tungsten fibre was produced that had a tensile strength of 312,000—345,000 psi.

The apparatus of FIGS. 1-3 could readily be adopted for plating glass filament. Since glass is not electrically conducting, it cannot be heated by self-resistance. Accordingly, a suitable pre-heater, such as a resistance, would be required to heat the glass to a temperature to cause decomposition of the liquid reactant upon contact.

The silicon carbide coated filaments of the type described could be used to satisfy the current need for lightweight, high strength and high modulus fibres for use in wound structures as well as in fibre reinforced structures.

The use of extremely fine glass as a substrate in the practice of this invention results in a thin filament, e.g., one having a total diameter between one or two mils with properties far superior to those of the uncoated glass. Glass is especially useful because it is possible to make extremely fine filaments of this material, which intrinsically has a low density. Fine diameter fibres of silicon coated glass filaments produced in accordance with this invention are easy to handle in wrapping or winding applications, and have extremely high strength and modulus to weight ratios. Especially suitable as a substratum for the preparation of fine silicon carbide coated glass filaments in accordance with this invention is "E" glass yarn. The glass should be pre-heated well above the decomposition temperature of liquid reactants described herein so as to make it possible to maintain it for a sufficient period of time at decomposition temperature in the deposition chamber.

This technique can be extended to provide a high speed, efficient system for coating glass fibre or yarn with silicon carbide. Thus, instead of providing a separate furnace for preheating the already formed glass, the deposition chamber may be placed below the exit orifice of a glass filament producing furnace or spinnerette. The glass emerging from either the furnace or spinnerette is thereby already hot enough for deposition to take place. Such a procedure greatly simplifies the entire system and allows the silicon carbide to deposit as part of the glass forming process. In the case of yarn, placing the furnace below the spinnerette but in front of any gathering device, allows for coating of the filaments before gathering, thereby insuring complete and uniform coating of each filament in the yarn.

An apparatus suitable for carrying out such an embodiment of the invention is shown in FIG. 4. In FIG. 4, 100 represents a suitable spinnerette into which is fed molten glass 101 at temperature and pressure conditions well known to the art. The hot glass filaments 102 emerge from the spinnerette directly into reaction chamber 104 which is filled to a suitable level with a silicon carbide source compound 106 of the type described herein. A suitable heat exchanger mechanism 108 surrounds the chamber 104 to keep the reactant liquid at desirable temperature. The filaments 102 pass

through the fluid reactant 106 and are coated with a silicon carbide in accordance with the teachings contained hereinabove. If desired, a suitable gathering device 109 may be provided to gather the glass filaments 102 into a yarn. The yarn gatherer 109 is provided with a suitable sealing device 110, e.g., a mercury seal, to prevent loss of source compound 106 from the reaction chamber. The gathered glass yarn 112 may be stored on a suitable storage device, for example, reels. If desired, the source compound used with the apparatus of FIG. 3 could be gas, although it should be understood that in the preferred embodiment, liquid source compound would be used. In the embodiment wherein gas is used as the reactant, the heat exchanger 108 would be utilized to maintain the reactant in a gaseous state 15 and to prevent loss of heat from filaments 102.

It should be pointed out that the coating rates of this invention are very high when liquid source compound is used, so that even though the substratum, e.g., glass filament, is rapidly cooled below the deposition temperature upon contact with the liquid source compound, it will be coated with a thin layer of silicon carbide.

The silicon carbide source compound for use herein may be any suitable organosilicon halide corresponding to the formulae:



wherein R is an alkyl, aryl or alkyl aryl radical, and X is halogen, i.e., chloride, bromide, fluoride or iodide, including mixtures of such compounds.

Preferred for use are the lower alkyl (i.e., less than 8 carbon atoms) dichloro and trichloro silanes, such as methyl dichlorosilane, methyl trichlorosilane, ethyl dichlorosilane, ethyl trichlorosilane, and the like. Also may be mentioned phenyl trichlorosilane and phenyl dichlorosilane. When the lower alkyl silicon halides referred to are employed, the surface in contact therewith will be heated to between about 500° and 1,500°C., preferably between about 800° and 1,500°C.

The reaction chambers suitable for use in carrying out the processes of the invention can be constructed entirely of glass or quartz, or metal, or partly of each of these materials. Ordinarily, the reaction will be carried out under atmospheric pressure, although operation under pressure is also contemplated.

The invention is particularly suitable for imposing a thin, adherent, non-porous oxidation and corrosion resistant silicon carbide coating on base metals such as columbium, tantalum and tungsten, which are vulnerable to oxidation at high temperature and which will fail rapidly if not protected by a suitable coating. Such metals or alloys thereof, and particular alloys containing one or more of the foregoing, are useful as vanes for gas turbines, especially jet aircraft engines. Other substrates which may be advantageously coated with silicon carbide in accordance with this invention are those which have a melting point exceeding the formation temperature of silicon carbide and include molybdenum, rhenium, silicon, carbon, glass, alumina, graphite and the like.

It should be understood, however, that using the teachings contained herein it is possible to coat liquid substrata, e.g., liquid drops or droplets or globules, by contacting them with the liquid organosilanes described. In FIG. 4, outlets 117 and 118 may be used to

feed or circulate reactant 106 to the reaction chamber 104.

The invention in its broader aspects is not limited to the specific details shown and described, but departures may be made from such details within the scope of the accompanying claims without departing from the process of the invention and without sacrificing its chief advantages.

What is claimed is:

1. A method for depositing a thin, adherent oxidation and corrosion resistant silicon carbide coating on a filamentary base material to produce a structural composite filament which comprises:  
selecting a filamentary base material which has a melting point which exceeds the formation temperature of silicon carbide; and  
continuously passing a hot surface of the filamentary base material through liquid organosilicon halide, the temperature of said hot surface being sufficiently high to cause the organosilicon halide immediately surrounding said hot surface to film boil, decompose, and deposit on said filamentary base material an adherent coating of oxidation and corrosion resistant silicon carbide.
2. The method of claim 1 wherein the base material is an electrical conducting material which is heated by electrical resistance heating above the decomposition temperature of the organosilicon halide while in contact with the liquid organosilicon halide.
3. The method of claim 1 wherein the base material is an electrical insulating material, which is pre-heated to a temperature above the decomposition temperature of the organosilicon halide prior to contact therewith.
4. The method of claim 1 wherein the organosilicon halide is a lower alkyl silicon chloride.
5. The method of claim 4 wherein the temperature of the base material in contact with the liquid organosilicon halide is between about 800° and 1,500°C., and wherein the organosilicon halide is a member selected from the group consisting of methyl dichlorosilane, methyl trichlorosilane, ethyldichlorosilane and ethyl trichlorosilane.
6. The method of Claim 1 wherein the base material is a member selected from the group consisting of tungsten, tantalum, columbium, alloys containing one of the foregoing, and alloys of the foregoing.
7. The method of Claim 1 wherein the base material is an insulating material selected from the group consisting of glass and alumina.
8. The method of Claim 1 wherein the base material is a glass filament having a diameter of less than about 2 mils.
9. A method of depositing silicon carbide on a wire comprising the steps of immersing a wire in an organic liquid chemically including silicon and carbon, heating said wire until said liquid boils vigorously and film boiling is achieved, and maintaining said film boiling for a period of time thereafter, said wire being an electrically conductive wire and having a melting point such that said film boiling can be maintained for a period of time sufficient to deposit a desired coating of said silicon carbide on said wire, said organic liquid containing a compound selected from the group consisting of methyl trichlorosilane, methyl dichlorosilane, ethyl trichlorosilane and ethyl dichlorosilane.

10. The method of claim 9 wherein said heating is effected by passing an electrical current through said wire.

11. The method of claim 10 wherein said wire is metal, metal alloy or graphite.

12. The method of claim 11 wherein said wire is tungsten.

13. A method of depositing silicon carbide on a wire comprising the steps of immersing a wire in an organic liquid chemically including silicon and carbon, heating said wire until said liquid boils vigorously and film boiling is achieved, and maintaining said film boiling for a period of time thereafter, said wire being an electrically conductive wire and having a melting point such that film boiling can be maintained for a period of time sufficient to deposit a desired coating of said silicon carbide on said wire, said organic liquid containing a compound selected from the group consisting of organosilicon halides defined by the formulae



wherein R is a lower alkyl radical and X is chlorine.

14. The method of coating an object with silicon carbide which consists of:

heating said object to at least 1,150°C; and then quenching said object in a liquid bath consisting essentially of one or more members chosen from the

20

25

30

35

40

45

50

55

60

65

group of silanes having the general formula



wherein each R is a member of the group consisting of chlorine and hydrogen and R<sub>1</sub> is a member of the group consisting of methyl, ethyl and propyl groups.

15. The method of coating an object with silicon carbide which comprises:

heating said object to at least 1,150°C; and then immersing said object in a liquid bath consisting essentially of one or more members chosen from the group of silanes having the general formula



wherein each R is a member of the group consisting of chlorine and hydrogen and R<sub>1</sub> is a member of the group consisting of methyl, ethyl and propyl groups.

\* \* \* \* \*